

## UNITED STATES PATENT OFFICE.

CHRISTIAN JOHN WERNLUND, OF TOTTENVILLE, NEW YORK, ASSIGNOR TO THE ROESSLER & HASSSLACHER CHEMICAL COMPANY, OF NEW YORK, N. Y., A CORPORATION OF NEW YORK.

## METHOD AND ANODE FOR ELECTRODEPOSITION OF RUST-RESISTING COATINGS.

No Drawing.

Application filed January 5, 1924. Serial No. 684,506.

To all whom it may concern:

Be it known that I, CHRISTIAN JOHN WERNLUND, a citizen of the United States, and resident of Tottenville, in the county of Richmond and State of New York, have invented certain new and useful Improvements in Methods and Anodes for Electrodeposition of Rust-Resisting Coatings, of which the following is a specification.

10 My invention relates in general to the electroplating on iron and steel or other metal articles of alloys of cadmium and mercury.

Cadmium has many properties which render it advantageous over other metals and alloys as a protective coating for metals such as iron and steel. It is light in color and has a higher solution potential than iron, thus tending to protect the iron from 15 corrosion. As its solution potential is higher than that of iron and lower than that of zinc, the same weight of protective coating of cadmium affords more protection to atmospheric corrosion than is afforded by straight zinc. Also more cadmium than zinc can be deposited per unit of current used. The oxide coating formed by atmospheric or other corrosion of cadmium is 20 thinner and more adherent than that formed on zinc, consequently the tendency of cadmium to scale off and waste away is much less pronounced than that of zinc.

While I have found that pure cadmium coatings can be effectively deposited electrolytically, I have further found that alloy coatings comprising cadmium retain in large measure the advantageous features of pure cadmium coatings in durability and rapidity of deposit and can be much more 25 cheaply and conveniently produced than previous coatings of pure cadmium. According to my invention, I produce alloyed coatings comprising over 2% of cadmium and another metal, such as cadmium and mercury or zinc, or zinc, cadmium and mercury, using either plain anodes with a suitable bath, or alloy anodes, or both. The coatings have the enhanced practical advantages 30 characteristic of pure cadmium coatings in giving better protection than zinc with less thickness, good color of coating, and economy of current. The advantage of using mercury in combination with cadmium or

zinc and cadmium is that the resultant coating is more resistant to corrosion than 55 cadmium or zinc alone. The cathode potential is raised with consequent increased throwing power.

Such a coating may be formed by the use of a plating solution to which the proper 60 addition of cadmium or cadmium and mercury compounds soluble in the bath have been made, or the metals can be furnished to the solution by the use of cadmium 65 anodes or alloy anodes.

Examples of the scope of this invention are as follows:

## Example I.

To plate steel articles such as stampings 70 for aeroplane parts, I may proceed as follows:

The parts are first cleaned, preferably by sand blasting until all of the scale and loose dirt are removed. They are then put in a 75 hot alkaline cleaning solution containing from 1% to 5% of sodium hydroxide in order to preserve the clean surface.

The parts so cleaned are rinsed in water and suspended from the cathode rod into 80 a cadmium mercury alloy plating solution of the following composition:

|                  |        |            |
|------------------|--------|------------|
| Water            | 1 L.   | 1 gal.     |
| Sodium cyanide   | 60 G.  | 8 oz.      |
| Sodium hydroxide | 15 G.  | 2 oz.      |
| Cadmium hydrate  | 15 G.  | 2 oz.      |
| Mercuric oxide   | 0.1 G. | 0.0125 oz. |

Other conditions maintained are as follows:

Anodes, cadmium.

Temperature, 25° C. (77° F.).

E. M. F., 3 to 6 volts.

Current, 15 amperes per sq. ft.

An average analysis of the coating produced will show cadmium 98-99% and mercury 1-2%.

The various ingredients of the bath must be replenished from time to time as they become depleted.

## Example II.

I have found that a preferable method of stabilizing the cadmium and mercury contents of the bath is to use a cadmium mercury alloy anode to supply the desired quan-

tities of these metals to the solution. A preferred composition of such an alloy is cadmium, 98%; mercury, 2%.

5 In plating for example steel fittings for aeroplane parts, I proceed as in Example I, with the exception that in this case, the above mentioned alloy anodes are used. A coating of similar analysis to that in Example I is obtained.

10 In all the above examples the plating has been done in a still bath. It is understood that if mechanical solutions are used such as in barrel plating the concentrations of solutions, currents required, etc., may be 15 changed considerably to conform to the different operating conditions.

20 The elimination of any single component of the ternary alloy described above and in the following claims gives a binary alloy deposit either superior to straight zinc deposits or cheaper than straight cadmium.

25 I do not claim specifically herein the novel products resulting from the processes and baths herein disclosed, as such products are claimed in another application Serial No. 684,507, filed January 5, 1924.

What I claim is:

30 1. In cadmium electroplating from a cyanide bath, the step which consists in depositing cadmium in the presence of mercury to produce a coating of cadmium alloyed with a minor percentage of mercury.

35 2. Method of electroplating an alloy coating comprising cadmium and mercury which consists in making the article to be plated the cathode and providing an anode comprising cadmium and mercury.

40 3. Method of electrodepositing a cadmium alloy which consists in making the article to be plated the cathode and providing an

anode whose major constituent is cadmium the minor constituent being mercury.

4. Method of electrodepositing a rust resistant deposit of cadmium and mercury which consists in electrodepositing these 45 metals from a solution of their salts in an aqueous sodium cyanide sodium hydroxide solution wherein the article receiving the deposit is the cathode and an alloy of cadmium and mercury is the anode.

50 5. In cadmium electroplating from a cyanide bath the step which consists in depositing cadmium in the presence of mercury to produce a coating of cadmium alloyed with mercury.

55 6. In cadmium electroplating from a cyanide bath, the step which consists in depositing cadmium in the presence of a salt of mercury capable of resisting reduction by the bath to produce a coating of cadmium alloyed with mercury.

60 7. In cadmium electroplating from a cyanide bath, the step which consists in depositing cadmium in the presence of a salt of mercury capable of resisting reduction 65 by the bath to produce a coating of cadmium alloyed with a minor percentage of mercury.

70 8. An anode for electroplating comprising cadmium and mercury in amounts effective for the purpose set forth.

75 9. An anode for electroplating comprising cadmium and about 2% of mercury.

10. An anode for electroplating a major portion of which is cadmium and a minor portion is mercury.

Signed at Perth Amboy, in the county of Middlesex and State of New Jersey, this 28th day of December, A. D. 1923.

CHRISTIAN JOHN WERNLUND.